

# United States Patent

[11] 3,607,249

[72] Inventors **Fred C. Robertshaw**  
Cincinnati;  
**Jon L. Bartos, Loveland, both of Ohio**  
4,375

[21] Appl. No. 4,375

[22] Filed Jan. 20, 1970

[45] Patented Sept. 21, 1971

[73] Assignee The United States of America as  
represented by the United States Atomic  
Energy Commission

[51] Int. Cl. .... C22c 19/00

[50] Field of Search. .... 75/170,  
171; 148/32, 32.5, 158

[56] References Cited  
UNITED STATES PATENTS  
3,091,022 5/1963 Faulkner ..... 75/170  
Primary Examiner—Richard O. Dean  
Attorney—Roland A. Anderson

[54] **COBALT-IRON-TANTALUM HIGH-TEMPERATURE-STRENGTH ALLOY**  
1 Claim, 4 Drawing Figs.

[52] U.S. Cl. .... 75/170,  
148/32.5, 148/158

**ABSTRACT:** This invention covers a cobalt-base alloy consisting essentially of, in atom percent, 8-12 percent iron, 0.4 to 1.7 percent tantalum, and the remainder cobalt.



CREEP OF 3.2 Kg. VIM Co BASE ALLOYS AND TYPE 316 STN. STL.  
AT 750°C AND 1050 Kg/cm<sup>2</sup> (1500 psi) IN ARGON

FIG. 1

INVENTORS.

Fred C. Robertshaw

BY Jon L. Bartos

*Fred C. Robertshaw*

ATTORNEY.

PATENTED SEP 21 1971

3,607,249

SHEET 2 OF 4

CREEP OF 3.2 Kg VIM Co-BASE ALLOYS AND TYPE 316 STN. STL  
AT 650°C AND 1960 Kg/cm<sup>2</sup> (2800 psi) IN ARGON



Fig. 2

INVENTORS.  
Fred C. Robertshaw  
BY Jon L. Bartos

*Fred C. Robertshaw*  
ATTORNEY.



INVENTOR.  
Fred C. Robertshaw  
BY Jon L. Bartos

*Fred C. Robertshaw*

ATTORNEY.



Fig. 4

INVENTORS.  
 Fred C. Robertshaw  
 Jon L. Bartos  
 BY

*Roland A. Anderson*  
 ATTORNEY.

## COBALT-IRON-TANTALUM HIGH-TEMPERATURE-STRENGTH ALLOY

### BACKGROUND OF THE INVENTION

The invention described herein was made in the course of, or under, a contract with the U.S. Atomic Energy Commission.

The present invention relates to high-temperature-strength cobalt-base alloys having a substantially all-face-centered cubic (alpha) microstructure which is stable from room temperature up to the melting point.

In designing a cobalt-base alloy for use at high temperatures it is desirable to maintain the face-centered cubic structure throughout the temperature range from room temperature to in excess of the intended service temperature in order to eliminate the compromising alpha-to-epsilon phase change characteristic of elemental cobalt.

It is known that certain substitutional alloying additions to cobalt can promote or stabilize the face-centered cubic ( $\alpha$ ) phase. However, for maximum benefits, the alloy must not only exhibit phase stability, but should have a satisfactory combination of short and long term (creep) strength as well as ductility at room temperature as well as at high temperatures; specifically, a temperature in the range 550°-750°C.

### SUMMARY OF THE INVENTION

It is accordingly an object of the present invention to provide a cobalt-base alloy system which not only does not undergo phase transformation over a wide range of temperature, but which has a satisfactorily high combination of short term and long term strength to make the alloys particularly useful for service conditions at a temperature in the range 550°-750°C. This twofold object is met by providing a cobalt-base alloy containing sufficient amounts of iron to ensure the required alpha phase stabilization and sufficient amounts of tantalum to provide a practical combination of improved strength and ductility, rendering the alloy useful at temperatures in excess of 500°C. and as high as 750°C.

An examination of the cobalt-iron equilibrium phase diagram found in the literature will reveal that small amounts of iron will form a binary alloy stable in the alpha phase. In the present invention we find that from 8 to 12 percent iron will guarantee the existence of austenitic phase throughout the range of temperature from room temperature up to the melting point.

The present invention is predicated on the discovery that tantalum added to an alpha-stabilized cobalt-iron reference alloy combines to form a ternary-base system with a satisfactory combination of beneficial high-temperature properties. Addition of tantalum in stipulated amounts will provide a ternary alloy which is easily fabricable and as stable as the reference cobalt-iron binary system, but which has significantly increased short term and long term tensile properties at temperatures in the range 550°-750°C. The alloy system pos-

sessing this unique combination of properties is one consisting essentially of, in atom percent, 8 to 12 percent iron, from 0.3 to 2 percent tantalum, and the remainder cobalt. By the term "consisting essentially of" we mean to include alloying elements positively recited which critically determine the physical and mechanical properties of the alloy as well as residual amounts of other elements which are not deliberately added for any specific alloying purpose but which, nevertheless, accompany the alloy heat during its formation and the wrought

alloy during its fabrication into a desired part or shape. In general terms, such residual amounts of unstated impurities do not exist at more than the parts-per-million range with an approximate upper limit of no more than about 50 to 100 parts per million for each residual element.

The addition of tantalum to the reference cobalt-iron alloy to produce the aforementioned combination of satisfactory qualities is surprising from a number of standpoints. While recent work has indicated that tantalum raises the transformation temperature of cobalt, we find that it does not reverse the stabilizing effect of iron. Moreover, the addition of tantalum within the prescribed limits produces pronounced enhancement both in the short term and long term, i.e., creep, strength relative to the reference cobalt-(8-12) iron alloy. This effect is unique when it is considered that, while other ternary additives may be used to increase the short term strength of the binary alloy such as titanium, niobium, or molybdenum, they do not enhance creep strength to any satisfactory degree. Finally, the addition of tantalum within the prescribed limits provides an alloy which is easily prepared either by powder metallurgy or casting techniques. We prefer to form the alloy by vacuum casting in alumina crucibles under a vacuum of less than 1 micron because it leads to closer control of and reduces the amount of residual impurities. After the cobalt and iron in the crucible become molten, a partial pressure of argon is introduced, tantalum is added, and after a suitable molding period the resultant heat is poured into a copper mold. In our testing program all heats were extruded to 1.9 centimeters in diameter and converted to 0.076-centimeter thick sheet at rolling temperatures from 760° to about 1,200°C. Heating for forging, extrusion, and/or rolling operations were conducted in argon atmosphere. Tensile specimens were then prepared for testing. The crystal structures of all the cobalt-base alloys which were processed to form the tensile specimens were determined by X-ray diffraction techniques to be face-centered cubic.

The following description provides a summary of specific physical test data which characterize the novel Co-Fe-Ta system previously described in general terms.

### MATERIAL EVALUATION

#### Tensile Properties

Tensile testing was made on 0.076-cm. thick sheet specimens of a number of cobalt-iron-tantalum alloys in the as-rolled-and-aged (750°C.-20 hr.) condition. The results are indicated in the table below.

TABLE  
Tensile properties <sup>a</sup> of 3.2 KgVIM Co-base alloys

| Alloy heat No. | Composition, a/o | Test temp. <sup>b</sup> , °C. | Yield strength <sup>b</sup> |                      | Tensile strength |                      | Elong., percent |
|----------------|------------------|-------------------------------|-----------------------------|----------------------|------------------|----------------------|-----------------|
|                |                  |                               | K s.i.                      | Kg./cm. <sup>2</sup> | K s.i.           | Kg./cm. <sup>2</sup> |                 |
| M-433          | Co-9Fe           | RT                            | 18.7                        | 1,310                | 70.7             | 4,950                | 84.1            |
|                |                  | 550                           | 8.9                         | 620                  | 43.8             | 3,060                | 44.1            |
|                |                  | 650                           | 8.6                         | 600                  | 24.9             | 1,740                | 36.0            |
|                |                  | 750                           | 7.8                         | 550                  | 17.4             | 1,220                | 24.5            |
| M-406          | Co-9Fe-0.4Ta     | RT                            | 34.1                        | 2,390                | 71.2             | 4,980                | 68.7            |
|                |                  | 550                           | 20.0                        | 1,400                | 40.3             | 2,820                | 25.5            |
|                |                  | 650                           | 25.3                        | 1,770                | 35.3             | 2,470                | 16.7            |
|                |                  | 750                           | 23.8                        | 1,670                | 28.2             | 1,970                | 34.2            |
| M-446          | Co-9Fe-0.6Ta     | RT                            | 55.0                        | 3,860                | 88.2             | 6,170                | 44.3            |
|                |                  | 550                           | 44.2                        | 3,100                | 56.0             | 3,920                | 18.1            |
|                |                  | 650                           | 42.7                        | 2,990                | 51.0             | 3,570                | 20.6            |
|                |                  | 750                           | 38.0                        | 2,660                | 41.6             | 2,920                | 19.9            |
| M-445          | Co-9Fe-0.8Ta     | RT                            | 55.7                        | 3,900                | 90.4             | 6,320                | 48.9            |
|                |                  | 550                           | 41.5                        | 2,900                | 58.3             | 4,080                | 16.6            |
|                |                  | 650                           | 47.4                        | 3,340                | 56.6             | 3,960                | 17.9            |
|                |                  | 750                           | 42.8                        | 3,000                | 47.8             | 3,340                | 17.1            |

TABLE—Continued  
Tensile properties of 3.2 KgVIM Co-base alloys

| Alloy heat No. | Composition, a/o | Test temp., <sup>a</sup><br>°C. | Yield strength <sup>b</sup> |                      | Tensile strength |                      |         |
|----------------|------------------|---------------------------------|-----------------------------|----------------------|------------------|----------------------|---------|
|                |                  |                                 | K s.i.                      | Kg./cm. <sup>2</sup> | K s.i.           | Kg./cm. <sup>2</sup> | percent |
| M-423          | Co-9Fe-1Ta       | RT                              | 90.2                        | 6,310                | 121.7            | 8,520                | 28.2    |
|                |                  | 550                             | 67.0                        | 4,690                | 78.4             | 5,480                | 11.9    |
|                |                  | 650                             | 64.6                        | 4,530                | 70.8             | 4,950                | 15.0    |
|                |                  | 750                             | 53.0                        | 3,710                | 58.2             | 4,070                | 20.0    |
| M-409          | Co-9Fe-1.7Ta     | RT                              | 91.7                        | 6,420                | 128.3            | 9,000                | 22.2    |
|                |                  | 550                             | 76.3                        | 5,340                | 91.6             | 6,410                | 7.2     |
|                |                  | 650                             | 71.5                        | 5,000                | 82.5             | 5,780                | 6.6     |
|                |                  | 750                             | 65.2                        | 4,660                | 71.7             | 5,020                | 5.4     |
| Type 316 SS    |                  | RT                              | 35.7                        | 2,500                | 83.2             | 5,830                | 72.5    |
|                |                  | 550                             | 16.0                        | 1,120                | 64.0             | 4,470                | 42.5    |
|                |                  | 650                             | 13.8                        | 970                  | 47.9             | 3,350                | 47.1    |
|                |                  | 750                             | 13.0                        | 910                  | 34.0             | 2,380                | 52.2    |

<sup>a</sup> Specimens were 0.076 cm. thick with a 0.63-cm.-wide reduced section and a 2.54-cm. gage length. The major axis of each specimen parallels the rolling direction. All specimens were annealed at 750° C. for 20 hours in argon (except where noted).

<sup>b</sup> Yield strength value is based on deflectometer measurement of total load train elongation and is approximate.

<sup>c</sup> All elevated-temperature testing conducted in argon.

<sup>d</sup> RT=room temperature.

Results show that all the ternary additions of tantalum are particularly effective in increasing the short term tensile strength of the reference Co-9Fe binary alloy. While the increase in strength effected by increasing the tantalum content is accompanied by a reduction in ductility, it is clear that a favorable balance of strength and ductility can be achieved within the range of 0.4 to 1.7 atom percent tantalum. It should be noted here that ternary additions of such metals as Nb, Mo, and Ti will also increase short term tensile strength of the resultant ternary alloys as compared to a reference Co-9Fe alloy, but, as will be seen, do not improve creep properties nearly as well as a tantalum addition.

#### Creep Rupture Properties

The vacuum-induction-melted cobalt-base alloys previously referred to were creep tested in the as-rolled-and-aged (750° C.—20 hrs.) condition at 650° C. with a load of 1960 kg./cm.<sup>2</sup> and at 750° C. with a load of 1,050 kg./cm.<sup>2</sup> in argon atmosphere. The results are illustrated in FIGS. 1 and 2, which reveal that the cobalt-iron-tantalum alloys are far superior in creep to those alloys which have niobium, titanium, and molybdenum as the ternary additives. For purposes of comparison, the creep curve for a 316 stainless steel (curve A) is also included since this alloy can be used at temperatures in the range 550° to 750° C. It is clear that the cobalt-iron-tantalum alloys are superior to 316 stainless steels at both temperatures.

#### Age-Hardening Effect

During the course of processing and testing of the cobalt-iron-tantalum system of the present invention we have discovered that additions of tantalum impart hardness upon suitable heat treatment involving a preliminary solid solution treatment, quenching, and final aging at a lower temperature. The results show that heat treatment at a temperature in the range 1,200° to 1,210° C. for 1 hour will dissolve virtually all of the secondary phase materials. Sheet specimens were then aged at temperatures in the range 550° to 750° C. for 1 hour and it was found that maximum hardness was achievable at an aging temperature of 650° C. for a period of about 50 hours. Hardness values then remain fairly constant. The change in hardness resulting from a typical solutioning and heat treatment at 650° C. for 50 hours is shown in the curves of FIG. 3. As with tensile strength it is seen that there is a direct relationship between the increase in hardness and the tantalum content of each alloy.

The effect of age-hardening in accordance with the solid

solutioning-aging two-step operation results in the formation of a secondary phase which has been identified by metallographic and electron microscopy studies as forming a fine precipitate randomly distributed with thin grains and aggregated in the grain boundaries. This secondary phase has been identified as cobalt-tantalum particles,  $\gamma'Co_3Ta$ , a predominant portion of which are in the range of about 100 to 200 angstroms in diameter. It is this secondary phase which is believed to impart additional strength and hardness to the ternary cobalt-iron-tantalum system as compared to the reference binary cobalt-iron alloy.

In summary, we have shown that the addition of tantalum to a reference cobalt-iron ternary alloy imparts a unique combination of strength-inducing qualities to the new ternary cobalt-iron-tantalum system. The new alloy is characterized in having a stable, face-centered cubic, crystallographic phase throughout the range of temperature from room temperature to melting, avoiding any difficulties involved in phase transformation. In addition, the alloy shows a favorable combination of short term and high-temperature tensile strengths combined with excellent creep resistance as well as imparting an increased measure of hardness to the reference cobalt-iron alloy. These improved physical qualities are apparently due to the formation of a stable cobalt-tantalum secondary phase uniformly distributed within a cobalt-iron matrix.

The improvement obtained in this new cobalt-iron-tantalum system has already been demonstrated in the foregoing presentation of short term tensile, creep, and hardness data. They are somewhat more graphically illustrated in the curve of FIG. 4, which is a Larson-Miller parametric representation of the rupture life of several cobalt-iron-tantalum alloys compared with a 316 stainless steel, an alloy which can be used at temperatures in the range 550° to 750° C. The curves very clearly show that the Co-9Fe-Ta alloys containing 0.4 to 1.7 atomic percent tantalum are more creep resistant than 316 stainless steel for high-stress, that is, from 25 to 50 k.s.i., high-temperature (550° to 700° C.) applications. Lower stresses up to 25 k.s.i. at higher temperature, 700° to 800° C., applications require cobalt-iron-tantalum alloys with tantalum contents of 1 percent or more in order to exceed the rupture life properties of 316 stainless steel.

All concentrations of the novel alloy disclosed in this specification are in terms of atom percent.

We claim:

1. A cobalt-base alloy consisting essentially of 8-12 percent iron, 0.4 to 1.7 percent tantalum, and the remainder cobalt.